

April 27, 1971

Y. VAGINAY

3,576,773

POLYESTER BASED FIBERS COMPRISING A NON-LINEAR BRANCHED  
ETHYLENE TEREPHTHALATE POLYMERS

Filed June 3, 1969



Fig. 1.

Inventor

Yves Vaginay

By  
Cushman, Darby & Cushman  
Attorneys

## 1

3,576,773

**POLYESTER BASED FIBERS COMPRISING A NON-LINEAR BRANCHED ETHYLENE TEREPHTHALATE POLYMERS**

Yves Vaginay, Lyon, France, assignor to

Societe Rhodiacaeta, Paris, France

Filed June 3, 1969, Ser. No. 829,954

 Claims priority, application France, June 4, 1968,  
 50,064

Int. Cl. C08g 17/04

U.S. Cl. 260--22

3 Claims

**ABSTRACT OF THE DISCLOSURE**

This invention provides novel polyester fibers which when formed into a fabric do not give rise to pilling or fibrillation, made by melt-spinning branched chain polyethylene terephthalate of specified viscosity characteristics, and having specified tensile strength.

This invention relates to polyester fibers and a process for their preparation.

Fabrics woven from yarns of polyester fibers derived from terephthalic acid and ethylene glycol have exceptional strength, abrasion resistance and pleat retention. However the development of the use of polyester fibers in loosely woven or knitted fabrics is restricted to a large extent by the problem of pilling. In fact, in these types of fabric the individual fibers tend to migrate towards the surface and to form fibrous globules or pills which cannot become detached because of the high abrasion resistance and tensile strength of the polyester, i.e. the rubbing forces are much lower than the force required to tear the polyester fibers holding the pill.

As it is very difficult to prevent migration of the fibers attempts have been made to lower the mechanical properties of the polyester fibers and to adapt their tensile strength to the rubber forces applied during normal wear. During wear, the abrasion progressively lowers the tensile strength until it corresponds to the rubbing forces and pill drops off.

It has been attempted to lower the mechanical properties of the polyester fibers using polymers of lower molecular weight. Unfortunately the reduction in the molecular weight of the polyester is accompanied by a reduction in the viscosity in the fused state and in industry it is very difficult to spin a polyester having a viscosity in the fused state at 285° C. of less than 600 poises without the fibers sticking together. It is therefore difficult to obtain a fiber suitable for normal commercial use.

Although many attempts have been made to lower the tensile strength by treating the yarn or the woven fabric they have always come up against practically insoluble problems of reproducibility.

The present invention provides oriented polyethylene terephthalate fibers which are easily accessible industrially and yarns of fibers which do not give rise to pilling. Accordingly this invention provides a polyester-based fiber having an elongation at break of greater than 15% and a tensile strength of 18 to 36 g./tex which comprises a branched polyethylene terephthalate having a specific viscosity of 0.47 to 0.72 and a melt viscosity of 600 to 2500 poises at 285° C.

The fibers of this invention may be used in the manufacture of woven or knitted fabrics which substantially do not form pills.

For woven fabrics fibers having a tensile strength of 26 to 36 g./tex and for knitted fabrics fibers of 18 to 25 g./tex are generally chosen.

Depending on the proposed use and on any fibers with

## 2

which they are mixed, the elongation of the fibers of this invention may vary within wide limits. When they are used in admixture with wool and cotton, fibers having elongations of 25 to 60% are chosen.

5 The products of this invention show very slight variations in tensile strength with elongation for a constant specific viscosity and a constant melt viscosity consequently the graph of the variation in tenacity with specific viscosity can be accurately constructed, taking into account the scatter in elongations normally observed in industrial production.

The other characteristics of the fibers of this invention are interdependent. For example, for an elongation of 35% the points representing fibres of this invention are located within the area ABCD of FIG. 1 of the accompanying drawing. On this diagram the segment AB corresponds to the polymers having a viscosity 600 poises and the segment DC to the polymers having a viscosity 2,500 poises. The fibers currently sold commercially correspond to points above the segment BC.

20 The fibers of this invention may be prepared by extruding, in the fused state a branched polyethylene terephthalate containing  $y/n-2$  to  $z/n-2$  equivalent percent of  $n$ -valent chain units where  $n$  is 3 or 4,  $y$  is 0.2 and  $z$  is 2 having a specific viscosity of 0.47 to 0.72 and a melt viscosity of 600 to 2500 poises and orienting the yarns thus obtained by stretching.

25 The polymers used to prepare the products of this invention are branched polyethylene terephthalates and may be prepared by incorporating a branching agent, having three or four groups capable of forming stable bonds, such as ester, ether or amide bonds with the acid or alcohol groups, into the monomer mixture.

The preferred branching agents are polyols such as trimethylolpropane, trimethylethane, pentaerythritol or glycerine; polyacids such as trimelic acid, trimellitic acid or anhydride or pyromellitic acid or anhydride; polyphenols such as phloroglucinol or hydroxyhydroquinone; amino acids and acid-alcohols such as hydroxyisophthalic acid or aminophthalic acid; 2,2-bis(4-epoxypropoxyphenyl)-propane or diethanolamine.

30 Depending on the method of polyester synthesis employed 0.2 to 2 mols percent of the trifunctional branching agent relative to the terephthalic acid, or the terephthalic acid derivative, are used. Amounts of the order of 0.1 to 1 mol percent are preferred.

35 The polyesters which may be used in the process of this invention are essentially derived from terephthalic acid, ethylene glycol and a branching agent. They can however contain a proportion, up to 10 mol percent, of another glycol containing an aliphatic, cycloaliphatic or aromatic group or hetero-atoms such as propanediol, butanediol, hexanediol, decanediol, dimethylpropanediol, cyclohexanedimethanol, cyclobutanedimethanol, xylene glycol, polyoxyethylene glycol of molecular weight less than 6,000, polytetrahydrofuran, another diacid such as adipic, sebacic, dodecanedioic, isophthalic or hexahydro- or terephthalic acid, or dimeric acids derived from linoleic acid.

40 These polymers are preferably prepared in the presence of the usual transesterification and polycondensation catalysts and may contain agents to improve their colour or heat stability such as phosphorus derivatives e.g. phosphorous acid, phosphoric acid, phenylphosphonic acid or triphenylphosphite. They can also be matted, for example by adding a suspension of titanium oxide.

45 The following examples illustrate this invention. In these examples the terms used have the following meanings:

50 Specific viscosity: the specific viscosity at 25° C. of the polyester as a 1% solution in ortho-chlorophenol;

Melt viscosity: the viscosity in poises of the fused mass measured at 285° C.;

Pilling: the pilling observed after 30 minutes of the so-called "Random Tumble Pilling Test" or "RTPT" (Standard Specification ASTM D 1,375-64), the index 1 being assigned to articles having large numbers of pills and index 5 to articles practically free from pills;

Fibrillation: the observed effect produced by abrasion of dyed articles at the points of maximum rubbing. The linear polyester fibers in fact have a tendency to split into fibrils when they are firmly held in a tightly woven article and to show the undyed core of the polyester thus producing a bleaching effect.

In the following examples, the pilling tests were carried out on fabrics of rather loose construction such as twill or knitted fabrics, while the fibrillation test was carried out on fabrics of tight weave such as plain sheeting.

#### EXAMPLE 1

The following are introduced into a transesterification apparatus equipped with a stirrer, a double heating jacket and a fractionation column:

|                        | Parts |
|------------------------|-------|
| Dimethyl terephthalate | 1,150 |
| Ethylene glycol        | 361   |
| Calcium acetate        | 0.805 |
| Antimony oxide         | 0.110 |
| Trimethyl trimesate    | 1.95  |

<sup>1</sup> I.e. 0.65 mol percent relative to mols of dimethyl terephthalate.

The mixture is heated and the methanol begins to distil at a temperature of 147° C. When the evolution of methanol ceases at 230° C., the excess glycol is distilled and the following are added to the reaction mixture:

|                                             | Parts |
|---------------------------------------------|-------|
| Phosphorous acid                            | 0.402 |
| Titanium oxide suspended in ethylene glycol | 5.75  |

The mixture is transferred to a polymerisation autoclave where the temperature is progressively raised to 270° C. while the pressure is reduced to 0.4 mm. of mercury. The polymerisation is stopped when the power absorbed in stirring of the autoclave corresponds to a melt viscosity at 285° C. of 800 poises. The specific viscosity of the polymer thus obtained is 0.55 and its melting point is 261° C.

This polymer is spun at 278° C. through a spinneret with 168 0.50 mm. diameter holes and the yarn is wound up at a speed of 900 meters per minute. No adhesion between the filaments is observed.

After assembling several yarns, the cable is stretched at 100 meters per minute in a sizing bath heated to 70° C., to a draw ratio of 4.03, and is then crimped in a crimping box and dried.

The cable is cut on a Converter type of apparatus into 90 mm. fibers having the following properties:

Gauge—3.3 decitex  
Tensile strength—25 g./tex  
Elongation at break—35%  
Shrinkage in steam at 130° C.—2%

so as to form a yarn of 40/1 count and with a right-hand twist of 630 (coefficient of twist 100), and this yarn is then woven into a twill fabric. The woven fabric is desized, heat-set, dyed in the presence of a carrier, singed, brushed and cropped in accordance with the usual processes.

When tested by the "Random Tumble Pilling Test" (ASTM D 1,375-64) it gives an index of 5 after 30 minutes, that is to say there is practically no pilling on the surface of the woven fabric.

It also possesses good pleat retention.

A standard polyester having a specific viscosity of 0.57 and a melt viscosity of 600 poises is spun under the same conditions. A large amount of adhesion between filaments, causing stretching defects so that the cleanliness of the final fiber is very poor, is observed.

The properties of this fiber are as follows:

Gauge—3.3 decitex

Tensile strength—35 g./tex

Elongation at break—35%

Shrinkage in steam at 130° C.—3.5%

A twill fabric of the type described above woven from this fiber is tested by the "RTPT" test; an index of 2.5 indicating the presence of many pills is obtained. This tendency to form pills for practical purposes can not be improved because the use of polymer or lower molecular weight gives melt viscosities of less than 600 poises, incompatible with good industrial spinning.

#### EXAMPLE 2

The cable obtained after assembly in Example 1 is stretched such that its elongation at break is 22%. Its properties are then:

Gauge—3.2 decitex

Tensile strength—28.5 g./tex

Elongation at break—22%

Shrinkage in steam at 130° C.—1.5%

It is mixed with wool in the proportions of 55/45 and a yarn of 40/2 count with a 475 right-hand simple twist (coefficient of twist 75) and a 600 left-hand doubling twist (coefficient 95) is produced. A plain fabric is produced with this yarn.

After heat setting this fabric is dyed a deep navy blue in the presence of a carrier. No fibrillation of this plain fabric is observed on wear.

On the other hand, standard polyester fibers of specific viscosity 0.57, stretched to give an elongation at break of 22%, and converted to a fabric under the same conditions as above, show considerable bleaching at the points of maximum rubbing due to fibrillation.

#### EXAMPLE 3

Mixtures as in Example 1 but containing 0.65 mol percent of trimethyl trimesate are polymerised until polymers of various specific viscosities are obtained. They are then spun as above and the fibers, after being mixed with wool under the conditions of Example 1, are converted into a twill fabric for measuring pilling and into a plain fabric for measuring the fibrillation. The results obtained are shown in the table below:

| Experiment Number | Specific viscosity | Melt viscosity (poises at 285° C.) | Gauge (decitex) | Tensile strength (g./tex) | Elongation at break | Woven fabric | Pilling RTPT | Fibrillation     |
|-------------------|--------------------|------------------------------------|-----------------|---------------------------|---------------------|--------------|--------------|------------------|
| 1-----            | 0.58               | 1,000                              | 3.3             | 26.5                      | 34                  | Twill-----   | 5            | Nil.             |
| 2-----            | 0.58               | 1,000                              | 3.2             | 30                        | 25                  | Plain-----   | 5            | Practically nil. |
| 3-----            | 0.66               | 2,000                              | 3.3             | 30                        | 37                  | Twill-----   | 4.5          | Nil.             |
| 4-----            | 0.68               | 2,500                              | 3.2             | 31                        | 34                  | do-----      | 4            | Nil.             |
| 5-----            | 0.68               | 2,500                              | 3.4             | 29.5                      | 55                  | do-----      | 5            | Nil.             |

This fiber is mixed with wool in the following proportions:

|           | Percent |
|-----------|---------|
| Polyester | 55      |
| Wool      | 45      |

In all cases the high melt viscosity permits excellent spinning and good stretching to give a fiber which does not adhere and is very homogeneous.

#### EXAMPLE 4

Polymers of different viscosities are prepared under

the conditions described in Example 1 but the trimethyl trimesate is replaced by 0.8 mol of trimethylolpropane per hundred mols of dimethyl terephthalate. The polymers are tested as above, with the following results:

| Experiment Number | Specific viscosity | Melt viscosity (poises at 285° C.) | Gauge (decitex) | Tensile strength (g./tex) | Elongation at break | Woven fabric | Pilling RTPT | Fibrillation     |
|-------------------|--------------------|------------------------------------|-----------------|---------------------------|---------------------|--------------|--------------|------------------|
| 1-----            | 0.57               | 1,200                              | 3.3             | 25                        | 39                  | Twill-----   | 5            | Nil.             |
| 2-----            | 0.57               | 1,200                              | 3.3             | 26.5                      | 24                  | Plain-----   | 5            | Practically nil. |
| 3-----            | 0.62               | 2,000                              | 3.4             | 27                        | 34                  | Twill-----   | 5            | Nil.             |
| 4-----            | 0.67               | 2,500                              | 3.3             | 29                        | 38                  | do-----      | 4.5          | Nil.             |

25 g./tex seems the lower limit of tensile strength for use industrially in the manufacture of woven fabrics.

#### EXAMPLE 5

The replacement of the 0.8 mol percent of trimethylolpropane used in Example 4 by 0.4 mol percent of pentaerythritol gives results similar to those of Example 4.

| Experiment Number | Specific viscosity | Melt viscosity (poises at 285° C.) | Gauge (decitex) | Tensile strength (g./tex) | Elongation at break | Woven fabric | Pilling RTPT | Fibrillation |
|-------------------|--------------------|------------------------------------|-----------------|---------------------------|---------------------|--------------|--------------|--------------|
| 1-----            | 0.57               | 1,250                              | 3.3             | 25.5                      | 33                  | Twill-----   | 5            | Nil.         |
| 2-----            | 0.66               | 2,500                              | 3.3             | 29                        | 31                  | do-----      | 4.5          | Nil.         |

#### EXAMPLE 6

Polyethylene terephthalates are prepared with 0.38 mol percent of various trifunctional branching agents, and the following pilling results are obtained on a twill fabric prepared described in Example 1.

| Experiment Number | Branching agent                 | Specific viscosity | Melt viscosity (poises at 285° C.) | Gauge (decitex) | Tensile strength (g./tex) | Elongation at break | Pilling RTPT |
|-------------------|---------------------------------|--------------------|------------------------------------|-----------------|---------------------------|---------------------|--------------|
| 1-----            | Glycerine-----                  | 0.54               | 630                                | 3.3             | 28                        | 37                  | 5            |
| 2-----            | Trimethylolpropane-----         | 0.54               | 600                                | 3.3             | 27                        | 40                  | 4.5          |
| 3-----            | Methyl hydroxyisophthalate----- | 0.54               | 650                                | 3.2             | 28                        | 33                  | 4.5          |
| 4-----            | Trimethyl trimesate-----        | 0.54               | 600                                | 3.3             | 29                        | 35                  | 4.5          |
| 5-----            | Glycerine-----                  | 0.67               | 1,850                              | 3.3             | 35                        | 39                  | 2.5          |
| 6-----            | Trimethylolpropane-----         | 0.67               | 1,950                              | 3.2             | 36                        | 32                  | 2.5          |
| 7-----            | Trimethyl trimesate-----        | 0.67               | 1,880                              | 3.4             | 35                        | 35                  | 3            |

The results are very similar regardless of the trifunctional compound used which indicates that if the compound introduced forms stable bonds it is the branching of the polyester chains which affects the mechanical properties and not the manner of branching.

#### EXAMPLE 7

Similarly, polyesters containing 0.55 mol percent of trimethylethylene are used as above, with the following results:

| Experiment Number | Specific viscosity | Gauge (decitex) | Tensile strength (g./tex) | Elongation at break | Pilling RTPT |
|-------------------|--------------------|-----------------|---------------------------|---------------------|--------------|
| 1-----            | 0.525              | 3.3             | 25                        | 33                  | 5            |
| 2-----            | 0.70               | 3.3             | 34                        | 36                  | 3            |

#### EXAMPLE 8

1 mol percent of branching agent is used to prepare a polyester under the conditions as described in Example 1. The reaction time required to obtain polymers of the desired specific viscosities is greatly reduced compared to that for the unbranched polymer. To achieve good reproducibility of preparation, it is necessary to reduce the amount of polycondensation catalyst to a very small proportion or to use less active catalyst than antimony oxide, such as salts or oxides of lithium, magnesium or cadmium.

Thus, using a mixture of dimethyl terephthalate, ethylene glycol, calcium acetate and phosphorous acid as in Example 1, and 0.008 part of antimony oxide, it is pos-

sible to prepare polyesters having a specific viscosity of 0.5 to 0.65 in the presence of 1 mol percent of trimethylolpropane, the titanium oxide being introduced in a proportion of 0.5 percent by weight relative to the dimethyl terephthalate. The polycondensation time required to obtain a polymer of a specific viscosity of 0.54 (melt vis-

cosity at 285° C. 1,050 poises) is 1 hour 55 minutes, and this ensures both good reproducibility between experiments and economical use of the apparatus.

This polymer is spun and stretched as in Example 1 and

then cut into 80 millimeter fibers having the following properties:

Gauge—3.3 dtex  
Tensile strength—22 g./tex  
Elongation at break—41%

This fiber is mixed with wool in the proportion of 55/45 and a yarn of 36/1 count and 540 right-hand twist (coefficient 80) is prepared. This yarn is knitted, heat-set and then dyed with a carrier.

When subjected to the pilling test the knitted fabric has an index of 4, which is excellent for this type of article. If the knitted fabric is subjected to brushing and cropping the index is then 5.

A knitted fabric obtained from a yarn of 40/1 count and coefficient of twist of 85, in a polyester/wool mixture in the proportion of 70/30, is rated as 3 in the same test, and as 4-5 after cropping and brushing.

A knitted fabric prepared from the standard polyester described in Example 1 and treated under the same conditions is rated as follows:

in a 55/45 mixture—index 1  
in a 70/30 mixture—index 1

#### EXAMPLE 9

Three polyesters of different specific viscosities are prepared under the conditions described in Example 8 from a monomer mixture containing 1.2 mol percent of trimethylolpropane relative to the dimethyl terephthalate.

When treated as described in Example 8, the following results are obtained:

state at 285° C. of 1,500 poises is obtained. Its specific viscosity is then 0.60. When spun and stretched under

| Experiment Number | Specific viscosity | Gauge (decitex) | Tensile strength (g./tex) | Elongation at break | Polyester/wool | Brushing and cropping treatment | RTPT rating |
|-------------------|--------------------|-----------------|---------------------------|---------------------|----------------|---------------------------------|-------------|
| 1                 | 0.49               | 3.3             | 19                        | 36                  | 55/45          | No-----                         | 5           |
| 2                 | 0.49               | 3.3             | 19                        | 36                  | 55/45          | Yes-----                        | 5           |
| 3                 | 0.49               | 3.3             | 19                        | 36                  | 70/30          | No-----                         | 4           |
| 4                 | 0.49               | 3.3             | 19                        | 36                  | 70/30          | Yes-----                        | 5           |
| 5                 | 0.60               | 3.3             | 22.5                      | 32                  | 55/45          | No-----                         | 4           |
| 6                 | 0.60               | 3.3             | 22.5                      | 32                  | 55/45          | Yes-----                        | 5           |
| 7                 | 0.60               | 3.3             | 22.5                      | 32                  | 70/30          | No-----                         | 3           |
| 8                 | 0.60               | 3.3             | 22.5                      | 32                  | 70/30          | Yes-----                        | 4           |

It can be seen from these results that by using a polyester of low specific viscosity (0.49) but of sufficient melt viscosity for good spinning (1,100 poises), when the polyester is mixed 55-45 with wool, it is possible to obtain, an article which without brushing or cropping is satisfactory from the point of view of pilling.

#### EXAMPLE 10

A polymer containing 1.6 equivalents of chain links derived from trimethylolpropane is prepared, spun, and knitted as above, and tested as a 70/30 mixture with wool.

the conditions described in Example 1, it has the following properties after being cut into 90 mm. fibers:

Gauge—3.3 dtex  
Tensile strength—24 g./tex  
Elongation at break—30%

20 It is spun, as a 55/45 mixture with wool, into 40/1 (count) and then woven into a twill fabric, and dyed in the piece, without a carrier, to give a deep shade. In the "RTPT" test the fabric gives an index of 5 after brushing and cropping.

| Experiment Number | Specific viscosity | Gauge (decitex) | Tensile strength (g./tex) | Elongation at break | Bushing and cropping treatment | RTPT rating |
|-------------------|--------------------|-----------------|---------------------------|---------------------|--------------------------------|-------------|
| 1                 | 0.49               | 3.3             | 18                        | 39                  | No-----                        | 4.5         |
| 2                 | 0.49               | 3.3             | 18                        | 29                  | Yes-----                       | 5           |
| 3                 | 0.57               | 3.3             | 19.5                      | 32                  | No-----                        | 4           |
| 4                 | 0.57               | 3.3             | 19.5                      | 32                  | Yes-----                       | 5           |

Using this proportion of crosslinking agent and a polymer of low viscosity, the 70/30 knitted fabric can be used without brushing or cropping.

#### EXAMPLE 11

The polymer prepared in Example 8 is spun and stretched to give individual fibers having the following properties:

Gauge—1.7 dtex  
Tensile strength—23 g./tex  
Elongation at break—29%  
Cut—40 mm.

These fibers are mixed with cotton in the proportion of 75/25, spun into 50/1 (count) with an 850 right-hand simple twist (coefficient 120) and woven in a taffeta weave. This taffeta is tested for pilling by the "RTPT" test. The following results were obtained.

Index  
After printing ----- 3  
After brushing, cropping and printing ----- 5

Under the same conditions a standard polymer of specific viscosity of 0.57 gives a woven fabric of index 1, which is very low.

#### EXAMPLE 12

The fiber of Example 11 is mixed with cotton in the proportion of 50/50 and spun into 50/1 (count) with a 915 right-hand twist (coefficient 130), and then knitted into gauge 20 interlock.

After heat-setting at 210° C. and bluing in a bath, the knitted fabric is "RTPT" tested and rated at 4, which is acceptable for this type of article.

#### EXAMPLE 13

A polyester which is branched with 0.8 mol percent of trimethylolpropane and which contains 6% by weight of polyoxyethylene glycol is prepared under the conditions described in Example 1 until a viscosity in the fused

40 An unbranched copolyester of the same specific viscosity has the following properties under the same conditions:

Gauge—3.2 dtex  
Tensile strength—36 g./tex  
Elongation at break—35%

45 The pilling test on a woven fabric prepared from this fiber gives a rating of 2.

#### EXAMPLE 14

This same fiber mixed with wool 70/30 and spun into 36/1 (count) is knitted and "RTPT" tested after setting and dyeing.

Without cropping and brushing, the knitted fabric is rated: 3-4  
After cropping and brushing, the knitted fabric is rated: 4-5

55 We claim:  
1. A polyester-based fiber having an elongation at break greater than 15% and a tensile strength of 18 to 36 g./tex, which comprises a non-linear branched ethylene terephthalate polymer containing 0 to 10 mol percent of ester structural units other than ethylene terephthalate units and  $y/n-2$  to  $Z/n-2$  equivalents percent of  $n$ -valent chain links, where  $n$  is 3 or 4,  $y$  is 0.2 and  $Z$  is 2, the remainder being ethylene terephthalate units, the said polymer having a specific viscosity of 0.47 to 0.72 as determined in a 1% solution thereof in ortho-chlorophenol at 25° C., and a melt viscosity of 600 to 2500 poises at 285° C.

2. A fiber according to claim 1 wherein the ethylene terephthalate polymer contains up to 10 mol percent of propanediol, butanediol, hexanediol, decanediol, dimethyl-propanediol, cyclohexane, dimethanol, cyclobutanediethanol, xylylene glycol, polyoxyethylene glycol of molecular weight less than 6000, polytetrahydrofuran, adipic acid, sebacic acid, dodecanedioic acid, isophthalic acid, hexahydroisophthalic acid, terephthalic acid, a

dimeric acid derived from linoleic acid or a mixture thereof.

3. A fiber according to claim 2 wherein the terephthalate polymer is branched with trimethylolpropane, trimethylolethane, pentaerythritol, glycerine, trimesic acid, trimellitic acid, trimellitic anhydride, pyromellitic acid, pyromellitic anhydride, phloroglucinol, hydroxyhydroquinone, hydroxyisophthalic acid, aminophthalic acid, 2, 2-bis(4-epoxypropoxyphenyl)-propane or diethanolamine.

## FOREIGN PATENTS

745,690 11/1966 Canada ----- 260—75

## OTHER REFERENCES

5 Youngson et al.: Journal Chemical Society, June 1950,  
pp. 1613—1622.

DONALD E. CZAJA, Primary Examiner

10 R. W. GRIFFIN, Assistant Examiner

## References Cited

## UNITED STATES PATENTS

## U.S. Cl. X.R.

|           |        |                     |         |               |
|-----------|--------|---------------------|---------|---------------|
| 3,033,827 | 5/1962 | Kibler et al. ----- | 260—77  | 8—179; 260—75 |
| 3,446,758 | 5/1969 | Wiener -----        | 260—2,3 |               |
| 3,446,766 | 5/1969 | Taylor -----        | 260—22  | 15            |